

## UNITED STATES PATENT OFFICE

WILHELM PUNGS, OF LUDWIGSHAFEN-ON-THE-RHINE, AND ERICH FRESE, OF NEU-ROESSEN, GERMANY, ASSIGNEES, BY MESNE ASSIGNMENTS, TO STANDARD-I. G. COMPANY, OF LINDEN, NEW JERSEY, A CORPORATION OF DELAWARE

## INCREASING THE VISCOSITY AND IMPROVING THE LUBRICATING PROPERTIES OF OILS

No Drawing. Application filed June 13, 1928, Serial No. 285,205, and in Germany June 25, 1927.

This invention relates to an improved process for increasing the viscosity and improving the lubricating properties of oils.

We have found that Montan wax, which has been bleached by oxidation, with chromic acid or the salts thereof, if desired, together with organic acids or sulphuric acid, for example, as described and claimed in Patent Nos. 1,690,876 and 1,699,250, is excellently adapted for considerably increasing the viscosity of oils especially tar oils, mineral oils and the like, or mixtures of the same, and for improving their lubricating properties to a large extent. An addition, for example, of even about 1 per cent or less of the wax so bleached is sufficient to lower the coefficient of friction of solid bodies by about 30 per cent of that obtained when unmixed oils are employed. By an addition of about 4 per cent and upwards, the viscosity of the said oils, and also of nearly all vegetable and fish oils, such as castor oil, rape oil, olive oil, sesame oil, cod-liver oil and the like, is increased to such an extent that products resembling and having the consistency of petroleum jelly and ointment are obtained, which are highly suitable for use in therapy and in cosmetics.

The property of rendering oils considerably more viscous by a very small addition of Montan wax bleached by oxidation as before mentioned, and of furnishing products similar to petroleum jelly and ointment by larger additions of the said agent is not displayed to the same extent either by crude Montan wax, Montan wax bleached in any other way, ceresine or carnauba wax.

According to the present invention, for example, an addition of one quarter per cent of bleached Montan wax raises the viscosity of a lubricating oil from 14.2 Engler degrees at 20° C. to 25.2 Engler degrees at 20° C., whereas, in the case of carnauba wax, an addition of 2 per cent, or eight times as much, is needed to produce the same effect. An addition of 7 per cent of Montan wax bleached as aforesaid to the same oil effects the formation of a mass of the consistency of ointment, with the dropping point 63° C. whereas the same amount of crude Montan wax only

raises the viscosity to 34.1 at 20° C. The dropping point is determined by heating the material to be considered in a tube, which is open at the bottom. The dropping point is the temperature, at which the first drop falls off from the bottom of the said tube.

The following examples will further illustrate the nature of the said invention which however is not limited thereto.

## Example 1

Lubricating oil with the viscosity of 19.3 Engler degrees at 25° C. is heated to about 100° C. and mixed, by stirring, with three quarters per cent of Montan wax bleached with chromic acid. When cold, the viscosity is found to have risen to 47.9 Engler degrees at 25° C. and the coefficient of friction lowered by about 30 per cent.

## Example 2

100 parts of paraffin oil are heated to 100° C. and mixed, by stirring, with 7 parts of Montan wax bleached by oxidation with chromic acid. The resulting paste is triturated when cold, and forms a white product, similar to petroleum jelly and with the dropping point 68.5° C.

## Example 3

Castor oil is heated to 120° C. and mixed by stirring, with 10 per cent of Montan wax bleached by oxidation with chromic acid. On cooling, a white product of the consistency of ointment and with the dropping point 73° C. is obtained.

What we claim is:—

1. A process for increasing the viscosity and improving the lubricating properties of oils, which comprises providing these with an addition of Montan wax bleached by oxidation with chromic acid.

2. A process for increasing the viscosity and improving the lubricating properties of oils, which comprises providing these with an addition of Montan wax bleached by treatment with chromic acid in the presence of an acid selected from the group consisting of the organic acids and sulphuric acid.

3. As compositions of matter, improved

viscous oils comprising an oil and Montan wax bleached by treatment with chromic acid.

4. As compositions of matter, products having the consistency of petroleum jelly and ointment comprising an oil and at least about

5 4 per cent of Montan wax bleached by oxidation with chromic acid.

6. As compositions of matter, products having the consistency of petroleum jelly and ointment comprising an oil and at least about

10 4 per cent of Montan wax bleached by treatment with chromic acid.

11 6. As a composition of matter an improved lubricating oil comprising a lubricating oil and an addition of  $\frac{1}{4}$  to  $\frac{3}{4}$  percent of Montan wax bleached by oxidation with chromic acid.

12 7. As a composition of matter an improved viscous oil comprising an oil and Montan wax bleached by oxidation with chromic acid in the presence of acids selected from the class

13 20 consisting of organic acids and sulphuric acid.

In testimony whereof we have hereunto set our hands.

WILHELM PUNGS.  
ERICH FRESE.

23

30

35

40

45

50

55

60

65